

## UNITED STATES PATENT OFFICE

2,189,264

## FERROPRUSSIAN PHOTOREPRODUCTION

John Holden, Reddish, Stockport, England, assignor to Keuffel & Esser Company, Hoboken, N. J., a corporation of New Jersey

No Drawing. Application November 30, 1937,  
Serial No. 177,321. In Great Britain December  
4, 1936

8 Claims. (Cl. 95—6)

This invention has reference to the production of light sensitive printing paper of the kind commonly referred to as "blue prints" and has for its object to provide improvements in such papers whereby the production of prints shall be more convenient than at present in that prints can be produced with a rapid exposure and a quick development by water or an aqueous solution without the usual washing, thus eliminating loss of time spent in drying, and the prints so produced have stabilised lines and background, and a controlled intensity of blue effected in the development and not requiring subsequent treatment to effect their ends.

According to this invention light sensitive printing paper of the kind referred to is made by sensitising the paper with solution containing a salt of iron in the ferric state, preferably a double salt with an alkali of an organic acid; a ferro-cyanide with or without a ferri-cyanide; a suitable buffer salt in neutral or alkaline condition; a fixing agent or agents being applied to the sensitised coating in whole or in part before or after exposure to light, such fixing agents being capable of rendering insoluble the ferro-cyanide and the ferri-cyanide, when in contact with water but being chemically separated from the cyanides if applied before exposure to light; intensifying or stabilising agents may also be applied under the same conditions as the fixing agents, the paper being developed by water or aqueous solution contact as distinct from washing.

According to one manner of carrying out the invention a paper of the kind known in the art to be suitable for printing papers of this kind is coated with a sensitising solution containing a salt of iron in the ferric state, and preferably a double salt with an alkali salt of an organic acid such as ferric ammonium oxalate, and a suitable ferro-cyanide, such as potassium ferro-cyanide or a mixture of potassium ferro-cyanide and a ferri-cyanide such as a potassium ferri-cyanide, or if desired the ferro-cyanide may be used alone. The function of the ferro-cyanide is to give higher printing speeds, and also to allow a wider range of exposure. The solution also contains a buffer salt, which may preferably be an alkaline oxalate, citrate or tartrate; acids must not be present. Photosensitive papers of the above type may be termed ferroprussiate papers.

Agents for fixing, stabilising or intensifying the print to be made on the paper are used and agents for all these purposes, or for any of these

purposes, may be applied or added in whole or in part to the paper before its exposure to light and subsequent development by contact with water or by an aqueous solution. If however, any of these agents are applied before the exposure of the paper precautions must be taken to prevent any reaction between them and the sensitised surface before such exposure to light takes place, thus ensuring that such agents can only enter into their desired chemical reaction when water or an aqueous developer is applied. If by mischance the paper should come into contact with water or aqueous solution or should become wet before exposure it will be spoiled; except by accidents or carelessness such contact does not occur.

In some instances the whole of one or more of such agents which may be required may be applied to the paper before exposure to light, and in other instances part only may be applied, the required balance being applied after exposure, or in other instances the whole of some, and part of the other agents may be applied before or after exposure.

Where the agents are not on the paper before exposure precautions must be taken to ensure the complete fixing of the print according to the thickness and type of the paper such as by treating the paper more than once with the developing solution either on the front or back or both, such treatment being however distinct from washing.

Agents which can be used for fixing or forming the insoluble salts with the ferro- or ferri-cyanides, but which do not constitute a complete list and which may not all be equally effective in every instance are metallo organic salts such as zinc, nickel, cobalt salts or aliphatic or aromatic acids, such as zinc salts of naphthalene sulphonic acids, or zinc salts of phenol sulphonic acids or certain metallic salts of the sulphuric acid esters of high fatty alcohols or the corresponding salts of the other metals named or of other metals which will form insoluble or non-reactive ferro- or ferri-cyanides.

There may also be used salts of inorganic acids of similar metals soluble in water e. g. zinc, nickel, cobalt sulphates or insoluble or slightly soluble salts, e. g. the oxides, carbonates or similar insoluble salts of metals which will form insoluble ferro- and/or ferri-cyanides or ferri-cyanides or non-reactive compounds thereof.

Oxidising agents to act as intensifying and stabilizing agents may be bichromates, persulphates, stabilised compounds of hydrogen perox-

ide, chloramines, hypochlorites, salts of para-dichlorosulphonamino benzoic acid. Certain oxidising agents may also have the property of forming insoluble or non-reactive salts with the ferro- or ferri-cyanides as well as acting as intensifying and stabilising agents to the background e.g. metallic peroxides, persulphates, chromates and double salts with the alkali persulphates or hypochlorites.

10 A wetting agent may be used if desired and to counteract or destroy its effect at any convenient stage a metallic salt may be used, such salt being one that will form an insoluble salt with the wetting agent e.g. barium salt.

15 Papers made according to this invention are easily developed by contact with a film of water or a developer in aqueous solution.

While papers according to this invention have been referred to as "blue prints" they are usually, 20 though not necessarily, deep blue and clear white prints; cream or yellow lines can be made; the term "blue print" is however used to distinguish this branch of the art from the production of "diazotype" papers.

25 The invention may be carried out in various ways of which the following are examples.

#### EXAMPLE I

30 A suitable paper is coated with a solution of the following composition:

##### Part A.—To a volume of 2,000 ccs.

50% solution ferric ammonium oxalate ccs 800  
35 Borax gms 50

##### Part B.—To a volume of 2,000 ccs.

20% solution potassium ferro-cyanide ccs 700  
25% solution potassium oxalate (neutral) ccs 500  
40 30% solution potassium ferri-cyanide ccs 100  
20% solution gum arabic ccs 100  
Cane sugar gms 400

45 Part A is added to Part B. Final volume 4,000 ccs.

The coated paper is dried and after exposure to light under a design is developed by the application of a thin film of a solution of the following composition:

50 Zinc sulphate crystals gms 50  
Magnesium sulphate crystals gms 50  
Mono-sodium-ortho-phosphate crystals gms 50  
55 Ammonium persulphate gms 15  
Wetting agent per cent 1 to 2  
Water to a final volume of 500 ccs.

The developing solution is conveniently applied 60 by contact with a roller rotating in a bath of the solution. Prints with white lines on a bright blue background are obtained which are stable towards light. The zinc sulfate acts as a fixing agent for the iron-cyanogen radicals, the magnesium sulfate and the oxidizing agent, persulfate, stabilizes and intensifies the blue background and the phosphate fixes the iron salts.

#### EXAMPLE II

70 In the following example the agent used to form the insoluble ferro- and ferri-cyanides is applied to the surface of the paper in the form of a fine dry powder before exposure to light.

75 A suitable paper is coated with the light sensitive solution described in Example I and dried,

the dry sensitized surface is then dusted with a fine dry powder of the following composition:

|               | Grams |
|---------------|-------|
| Zinc chromate | 20    |
| Zinc sulphate | 80    |

Excess of powder is removed by suitable means such as a brush rotating at high speed. Papers so obtained after exposure to light under a design are developed by the application of a thin 10 film of a solution of the following composition.

|                             |          |        |
|-----------------------------|----------|--------|
| Magnesium sulphate          | gms      | 50     |
| Mono-sodium-ortho-phosphate | gms      | 75     |
| Wetting agent               | per cent | 1 to 2 |

Prints in bright yellow lines which bleach to cream or white on exposure to light, on a stable blue background are obtained.

Part or whole of the wetting agents may be included in the dry powder.

Part or whole of one or the other agents used in the developer may be applied in the dry powder, and when all are applied in powder form, the print is developed by contact with a film of water.

The powdered composition may be applied to the back or unsensitized side if very thin e.g. 30 gram papers are used, or if a thick, absorbent paper is used it is treated in such a manner as to ensure that the necessary chemical reaction will 30 take place.

When powdered agents are to be applied to the surface of the paper, it has been found that the best results are obtained with a matt or semi-matt paper. Smooth papers generally do not give the 35 best results.

#### EXAMPLE III

In the following example the agent used to form the insoluble ferro-cyanide or ferri-cyanide is applied before exposure to light in non-aqueous solution.

A suitable paper is coated with the light sensitive solution described in Example I and dried. The dry paper is then coated on the sensitive side, or if the paper is absorbent on the reverse side 45 with a 10% alcoholic solution of a zinc salt of naphthalene sulphonic or disulphonic acid, and the alcohol is removed by drying in a current of warm air. Paper so prepared, after exposure to light under a design is developed by the application of a thin film of a solution of the following 50 composition:

|                             |          |        |
|-----------------------------|----------|--------|
| Magnesium sulphate          | gms      | 50     |
| Mono-sodium-ortho-phosphate | gms      | 75     |
| Ammonium persulphate        | gms      | 20     |
| Wetting agent               | per cent | 1 to 2 |

Water to a final volume of 500 ccs.

Prints with white lines on a stable bright blue background are obtained.

Salts of other metals such as manganese, nickel with inorganic or organic acids if soluble in a non-aqueous solvent may be used in place of zinc but may not be equally effective in every case.

The non-aqueous solution may, if desired, contain the whole or a portion of the wetting agent and/or buffer agents.

#### EXAMPLE IV

In the following example the agent used to form the insoluble ferro- and ferri-cyanide is applied before or after sensitising on the back of the paper. Colloids may be used to prevent penetration of a thin paper, or wetting agents may be used to assist penetration of thick or hard

surface paper. Contact of the reacting agents after exposure under a design is made by penetration of the paper, and a wetting agent may be used to assist this.

5. A suitable paper is coated with the light sensitive solution described in Example I and dried. The reverse side is then coated with a solution of the following composition:

|                             | Grams |
|-----------------------------|-------|
| 10 Zinc sulphate            | 200   |
| Mono-sodium-ortho-phosphate | 200   |
| Magnesium sulphate          | 200   |
| Dextrine                    | 200   |

made up to 1000 ccs. water and is again dried.

15. After exposure to light under a design the print is developed by the application of a film of developer, preferably applied to the sensitive side, of the following composition.

|                                     |           |        |
|-------------------------------------|-----------|--------|
| 20 Ammonium persulphate             | gms.      | 20     |
| Wetting agent (preferably volatile) | per cent. | 2 to 3 |
| Water                               | ccs.      | 500    |

25 Prints having white lines on a bright blue background are produced.

While as herein described the oxidising agent may also be a stabilising agent or line fixing agent, the oxidising agent does not necessarily perform the function of a stabilising agent, and a separate stabilising agent may be used instead of, or in addition to, the oxidising agent.

30 Suitable stabilising agents are buffer salts e. g. the acid or neutral phosphates of the alkali metals or ammonia, or salts of organic acids such as phthalic, benzoic, or their equivalents, or calcium or magnesium salts e. g. calcium chloride or magnesium sulphate.

What I claim as my invention and desire to secure by Letters Patent is:

40. 1. A light sensitive printing paper having a sensitized coating formed of a solution containing a salt of iron in the ferric state, a ferro-cyanide, a suitable buffer salt, a fixing agent comprising zinc salts of aliphatic acids applied to the sensitized coating and capable of rendering insoluble the ferro-cyanide when in contact with water but chemically separated from the cyanide before exposure to light, and a stabilizing agent applied to the coating, the coated paper being capable of 45 development by contact with water as distinct from washing.

2. A developer for solution in water to fix the unreacted color forming components of a ferro-

prussiate light sensitive layer, stabilize and intensify the color forming components, comprising a salt of a metal which forms insoluble iron-cyanogen compounds, a phosphate, an oxidizing agent for iron cyanogen compounds and a magnesium salt.

5. 3. A developer for the semi-dry development of ferroprussiate printing papers which developer comprises the combination of a soluble magnesium salt and the soluble salt of a metal selected from the group consisting of zinc, nickel and cobalt which salts when applied to an exposed ferro-prussiate light sensitive layer act in combination to stabilize the blue background against the action of actinic light.

10. 4. A developer for the semi-dry development of ferroprussiate printing papers which developer comprises the combination of a soluble magnesium salt and the soluble salt of a metal which reacts to form insoluble compounds with the iron-cyanogen radicals, which salts when applied to an exposed ferroprussiate light sensitive layer act in combination to stabilize the blue background against the action of actinic light.

15. 5. A developer for solution in water to fix the unreacted color forming components of a ferro-prussiate light sensitive layer, stabilize and intensify the color forming components, comprising an oxidizing agent, zinc sulfate, magnesium sulfate and mono-sodium-ortho-phosphate.

20. 6. The process for the semi-dry development of ferroprussiate papers comprising separately fixing the iron ion which has not reacted to form a compound which will be blue, and the iron-cyanogen radicals which have not reacted to form a compound which will be blue, which process includes separately applying a metal salt for insolubilizing the iron-cyanogen radicals and a phosphate for insolubilizing the iron ion.

25. 7. The method for stabilizing the blue background of a ferroprussiate print which is fixed by a metal salt comprising applying a solution of a magnesium salt thereto which is retained on the print.

30. 8. A developer for solution in water to fix the unreacted color forming components of a ferro-prussiate light sensitive layer, stabilize and intensify the color forming components, comprising a metallo organic salt the metal of which forms insoluble iron-cyanogen compounds, a phosphate, an oxidizing agent for iron-cyanogen compounds and a magnesium salt.

JOHN HOLDEN.